

May 30, 1944.

A. J. STAMM

2,350,135

WOOD IMPREGNATION

Filed Nov. 16, 1942

4 Sheets-Sheet 1

*Fig. 1.*



*Fig. 2.*



BY

INVENTOR  
A. J. STAMM

*A. J. Kramer*  
ATTORNEYS

May 30, 1944.

A. J. STAMM

2,350,135

## WOOD IMPREGNATION

Filed Nov. 16, 1942

4 Sheets-Sheet 2

Fig. 3.



Fig. 4.



INVENTOR  
A. J. STAMM

*H. G. Foss  
G. J. Kramer*  
ATTORNEYS

May 30, 1944.

A. J. STAMM

2,350,135

WOOD IMPREGNATION

Filed Nov. 16, 1942

4 Sheets-Sheet 3



*Fig. 5.*



*Fig. 6.*

*Fig. 8.*



BY

INVENTOR  
A. J. STAMM

*A. J. Stamm  
G. J. Kriamer*  
ATTORNEYS

May 30, 1944.

A. J. STAMM

2,350,135

## WOOD IMPREGNATION

Filed Nov. 16, 1942

4 Sheets-Sheet 4



BY

INVENTOR  
A. J. STAMM

ATLANTA  
H. D. Jones  
G. J. Kramer  
ATTORNEYS

## UNITED STATES PATENT OFFICE

2,350,135

## WOOD IMPREGNATION

Alfred J. Stamm, Madison, Wis., assignor to  
 Claude R. Wickard, as Secretary of Agriculture  
 of the United States of America, and his suc-  
 cessors in office

Application November 16, 1942, Serial No. 465,732

5 Claims. (Cl. 117—116)

(Granted under the act of March 3, 1883, as  
 amended April 30, 1928; 370 O. G. 757)

This application is made under the act of March 3, 1883, as amended by the act of April 30, 1928, and the invention herein described and claimed, if patented, may be manufactured and used by or for the Government of the United States of America for governmental purposes without the payment to me of any royalty thereon.

This invention relates to a process and apparatus for impregnating wood in the form of either a thin lumber or veneer. The wood may be either dried or in a green, water-soaked condition, and this invention concerns the impregnation of such wood with water-soluble solutes, such as, by way of illustration, stabilizing resins, fire-retardant chemicals, and toxic preservative chemicals. With respect to the dry woods, impregnation may be accomplished with various chemicals dissolved in organic solvents.

The principal object of this invention is to impregnate wood of the type mentioned by a process which is simple and quick as compared to those processes of the prior art, and which is adaptable to continuous operations as distinguished from batch operations.

According to the prior art, green veneer, and sometimes dry or partially dry veneer, is treated with water-soluble solutes by merely soaking the green or dry veneer in an aqueous solution of the solute. Although this process is simple, it is very time-consuming. For example,  $\frac{1}{8}$ -inch thick Douglas-fir veneer containing an amount of water equal to the dry weight of the wood (100 percent moisture content) will require about 14 hours' soaking at room temperature in a 50 percent aqueous solution of phenol-formaldehyde resin-forming mix to take up 30 percent of resin-forming solids on the basis of the dry weight of the untreated wood by diffusion into the wood structure.

When dry or partially dry wood is soaked in an aqueous solution, capillary absorption accompanies diffusion, but the combined processes are even slower than diffusion alone into veneer containing a large amount of water, as the effective liquid cross section through which diffusion takes place is materially reduced. For example,  $\frac{1}{8}$ -inch thick dry Douglas-fir veneer (6 percent moisture content) will require over 75 hours soaking to take up the same amount of resin-forming solids as are taken up by the aforementioned water-soaked Douglas-fir veneer in 14 hours.

It is desirable, therefore, from the standpoint of the rate of takeup of solute, to apply this

method to water-saturated rather than dry veneer. In this case, however, water must diffuse out from the wood as the solute diffuses in. When fresh solute is added to the treating bath to maintain the necessary outside concentration, the volume of the bath solution increases. It is hence necessary to remove part of the solution from the bath at intervals. The solute can be recovered from the removed solution in some cases by evaporating the water. In the case of the dimension-stabilizing, resin-forming systems, evaporation cannot be resorted to, as it causes premature curing of the resin. Treating water-saturated veneer by the diffusion method with such resin-forming mixes is hence wasteful of resin.

Both the rates of diffusion into wood and capillary absorption by wood can be increased by raising the temperature. The diffusion at 100° C. would, theoretically, be about four times that at 250° C., because of the change of temperature and the accompanying change in viscosity of the water. The capillary absorption would be increased about 2.6 times for the same temperature change because of the decreased surface tension and decreased viscosity of the solution. In cases where heating is not detrimental to the solution, it is found advantageous to heat the bath, but even then the takeup of solute is slow.

Immersing heated dry or partially dry veneer in the solution at room temperature aids capillary absorption because the air in the capillary structure which expanded on heating again contracts in the cooler solution, thus setting up a partial vacuum which aids capillary rise. A vacuum amounting to only  $\frac{1}{4}$  of an atmosphere can be obtained by heating the wood to 100° C. This will aid in taking up only a volume of liquid equal to one-fourth of the void volume of the wood.

Veneer can also be treated by dipping in solution, brushing a solution on the surface, or applying solution with a glue spreader. Sufficient solution for most purposes is taken up by the surface in one application only when the veneer is  $\frac{1}{40}$ -inch thick or less, or when the solution is quite viscous. When thicker veneer and low-viscosity solutions are used, it is necessary to dry the veneer and reapply the solution to the surface a number of times. This involves costly handling. When solutions of very high concentration are used to avoid multiple applications, diffusion is greatly retarded and hence the solvent tends to evaporate before the solute has an opportunity to diffuse completely into the structure.

The most rapid and efficient treating method now in use comprises increasing the rate and amount of capillary absorption by a vacuum, pressure, or combined vacuum-pressure method in a treating cylinder. Veneer of different species in thicknesses up to  $\frac{1}{8}$ -inch can be treated with an amount of solution equal to the weight of the wood in from 15 minutes to 4 hours by applying air pressures ranging from 20 to 75 pounds per square inch to the immersed veneer. This method of treating, although fairly rapid, requires expensive equipment, a great deal of handling of the material, and can only be operated on a batch basis.

Impregnating veneer by the method of the present invention overcome all the aforementioned deficiencies of the prior art. The method comprises passing veneer, which preferably has been preheated to make it plastic, between pressure rollers beneath the surface of the liquid with which it is to be impregnated. From the standpoint of preventing degradation of the veneer, it is preferable that the veneer sheets pass between the rollers at right angles to the axis of the rollers. This avoids injury to the wood and prevents curling of the sheets. It is desirable to compress the veneer to at least one-half the original thickness when an appreciable takeup of solute is desired. A large part of the air or moisture contained in the coarse-capillary structure is thus squeezed out. The veneer recovers very rapidly from the compression as the roller pressure is released, soaking in a volume of solution equal to the volume of air and water displaced. Besides the takeup of solution due to the mechanical treatment, there is an additional takeup resulting from the contraction of the air caused by the cooling of the hot veneer in the bath. To avoid having the temperature in the bath increase appreciably above room temperature, or any other desired point, by the hot veneer, cooling coils can be immersed in the bath near the compression rollers.

Green veneer, that is, veneer containing moisture above the fiber-saturation point (about 30 percent moisture content), which contains free water will tend to lose water while being compressed, and dilute the treating solution. To avoid this, veneer which contains free water should be compressed to about the same degree between another pair of rollers before entering the compression rollers of the treating bath so that the expressed moisture will not enter the bath. To aid in carrying away the expressed water and thus avoid reabsorption by the wood, a blast of hot air may be directed across each face of the veneer parallel to the axis of the rollers and as near the surface of the rollers as possible. In the case of dry, or partially dry veneer, containing moisture below the fiber-saturation point, it is unnecessary to subject the veneer to a predrying compression, so that only the treating bath rollers are necessary.

About half the void volume of  $\frac{1}{8}$ -inch thick air-dry veneer of different species can be filled with an aqueous solution in one minute or less by the method of this invention when the veneer is compressed to half its original thickness between the treating rollers, even when fairly viscous solutions are used.

Green, water-soaked veneer, as it comes from the cutter knives, can also be impregnated by the method of my invention by first passing the veneer through a pair of hot drying rollers to squeeze out a quantity of the free water, prior to

passing through the rollers of the treating bath. I have found that there is a tendency for the expressed water to be reabsorbed by the veneer, on the outlet side of the rollers, unless some means is provided. This surface water can be adequately removed by blowing air, preferably hot air, over both surfaces of the wood parallel to the axis of the rollers with the nozzle placed as near as possible to the line of emergence of the veneer from the rollers.

When appreciable amounts of free water remain in the veneer as it enters the impregnating solution, both the amount and rate of solution takeup are reduced. Green veneer should, therefore, be reduced to as near the fiber-saturation point as possible in the preliminary heating and compressing steps.

Although some species of wood will take up a sufficient amount of solution for most purposes by cold compression, there is a definite advantage in compressing the veneer while hot to avoid fiber rupture, to insure complete springback of the wood, and to aid penetration of the liquid by the contraction of the hot air in the wood structure as it cools in the solution. Compressing the wood while hot also reduces the work necessary to effect compression. Woods which tend to take up too much solution when compressed to half their original thickness should, when hot, be compressed to a lesser extent.

In the case of the more difficultly treated woods, it may be desirable to keep them immersed in the solution, after they pass through the rollers, for more than one minute, because the springback or recovery from the compression is somewhat slower. It is generally of no advantage to leave the veneer immersed in the solution for more than ten minutes.

Birch wood has a specific gravity which is about optimum for compression to half the original thickness. Denser woods cannot be compressed to this extent. Any attempt to do so would be disastrous to the equipment.

Woods which are readily compressed to half of their original thicknesses can be fed between rollers set to cause such compression. Light soft-wood veneers  $\frac{1}{8}$ -inch thick can be easily fed between rollers set to compress them to  $\frac{3}{16}$ -inch thick.

Most of the air removed from the veneer in the process of compression beneath the treating solution moves in the fiber direction through the veneer sheets and comes out at the ends of the sheets. Because of this, solution takeup occurs throughout the thickness of the veneer rather than just a fractional distance into the veneer from the faces. This is of value in reducing the subsequent storage time of the wet treated veneer to get a uniform distribution of the solute throughout the structure prior to drying. For example, veneers  $\frac{1}{8}$ -inch thick impregnated with Bakelite resinoid BR15,100 ordinarily require from 3 to 20 hours of aging, depending upon the veneers, under nondrying conditions (absence of heat and circulation) to permit them to come to practically complete swelling equilibrium.

In the accompanying drawings, there are illustrated suitable means for carrying out the methods described above, which, together with the following description, will more fully disclose this invention.

In the drawings:

Figure 1 is a plan view of an apparatus which may be used for impregnating the wood.

Figure 2 is a section along the line 2—2 of Figure 1.

Figure 3 is a section along the line 3—3 of Figure 1.

Figure 4 is a modified form of gearing for the compression rollers.

Figure 5 is a plan view of an apparatus for removing free water from green, water-soaked wood prior to impregnation.

Figure 6 is a section along the line 6—6 of Figure 5.

Figure 7 is a section along the line 7—7 of Figure 5.

Figure 8 is a section along the line 8—8 of Figure 5.

Referring with more particularity to the drawings, in which like numerals designate like parts, the apparatus illustrated in Figures 1, 2, and 3 comprises a tank 14 for holding the solution with which the wood is to be impregnated. The shape of this tank is preferably as illustrated, in the general form of a V, to economize on space, materials, and volume of treating bath. The lower end is provided with a drainage valve 12. The tank is supported by suitable frame members 13. One end of the tank is provided with a pair of compression rollers 14 and 15, between which the wood is compressed. The rollers are disposed so that the space between them is below the liquid level of the tank and so as to direct downward into the tank veneer passing therebetween.

The rollers 14 and 15 are preferably geared together to avoid slippage therebetween. In order to adjust the clearance between the rollers to permit the use of the apparatus with veneers of different standard thicknesses, the following means are provided: The bottom roller 15 is fixed to a shaft 16 which is rotatably mounted in bearings 17 and 18 on the sides 19 and 20 of the tank. The upper roller 14 is fixed to a shaft 21 which is rotatably mounted in bearings 22 and 23 movable in slots 24 and 25 in the sides 19 and 20 of the tank. The slots 24 and 25 are disposed above the liquid level and the bearings 22 and 23 are each provided with a pair of flanges 26 and 27 on either side of the slot, which can be drawn together by bolts 28 to secure the bearings in selected positions along the slots. The shafts 16 and 21 extend outward on one side of the tank and are provided with gearing units 29 and 30, respectively. The gearing unit 29 comprises a plurality of gears 31, 32, 33, 34, and 35 of different sizes, secured together and slidably mounted on and rotatable with the shaft 21 by means of a sliding key arrangement 35A or by any other suitable means. A collar 36, secured to the unit, is provided with a set screw 37 to secure the unit in different positions along the shaft. The gearing unit 30 is provided with the same number and sizes of gears 38, 39, 40, 41, and 42, respectively, but these gears are arranged in reverse order to those of the first unit. The unit 30 is attached to the shaft 16 for rotation therewith, substantially as shown. The shaft 16 is also provided with a pulley 43 for the transmission of power thereto by a belt 44 from a source of power, such as an electric motor 45. It is important to have the gears of the gearing units properly arranged in order to prevent locking. In gearing unit 29, the smallest gear 31 should be on one side and the next largest gear 35 on the other side. The next size gear 32 should be adjacent the smallest gear, and the next larger size gear 34 should be adjacent the gear 35, and so forth. In other words, the gears should be staggered on either side ac-

cording to their sizes. This staggered arrangement permits gears of equal sizes to be meshed with each other without any of the other gears meshing. By these means the rollers 14 and 15 can be geared to each other in a 1 to 1 relation with different amounts of clearance between them.

Another type of gearing is illustrated in Figure 4, and it embraces beveled gears 46 and 47, secured to the shafts 16 and 21, respectively. These beveled gears mesh with other beveled gears 48 and 49 mounted for rotation with a shaft 50 at right angles to the shafts 16 and 21. The shaft 50 is fixed to the frame of the machine by means of brackets 51 and 52. The gear 48 is fixed to the shaft 50, but the gear 49 is slideable thereon so as to mesh with the gear 47 in different positions of the roller 15. The movable gear 49 may be adjustably secured to the shaft 50 by means of a set screw 53 through a collar 54, integral with the gear. The shaft 50 is driven by power, delivered to a pulley 55 fixed thereto.

The ends of the shafts 16 and 21 on the extended sides are rotatably disposed in a fixed bearing 56 and a movable bearing 57, respectively, supported by a rigid bracket 58 secured to the tank. The bearing 57 is movable in a slot 59 of the bracket and is provided with flanges 60 and 61 and bolts 62, similar to the bearings 22 and 23.

Adjacent the fixed roller 14, there are disposed cooling units 63 in the tank for the purpose of carrying off heat from the liquid, imparted to it by the heated veneers. These coils are connected to a suitable source of cooling medium (not shown).

As the wood veneers are passed between the rollers 14 and 15, they descend into the liquid bath in the tank. Guide rollers 64 and 65 on the outside of the tank permit easier handling of the veneers and other guide rollers 66 and 67 placed within the tank keep the veneers in the solution for a sufficient period of time and direct them through the liquid bath so that one end comes up before the other. This makes it easier to withdraw the veneer from the bath.

When green, water-soaked veneer is used, it is necessary to give it a preliminary treatment for the purpose of expressing a portion of the free water therein. This may be accomplished by the apparatus illustrated in Figures 5, 6, 7, and 8, which comprises a suitable frame structure that carries a pair of hollow compression rollers 68 and 69. These rollers are adjustable with respect to each other, like the rollers 14 and 15, and are provided with similar means for this purpose. The various elements of such means are designated by numerals corresponding to like parts in Figures 1, 2, and 3.

Plane surfaces 70 and 71 are provided on either side of the rollers to support the veneers.

Shafts 72 and 73 and 74, 75, which support the rollers 68 and 69, respectively, are hollow to carry hot air through these rollers. Hollow shafts 72 and 74, on one side of the machine, are connected to the outlet pipe 76 of a hot-air generator 77 through a control valve 78 by means of sealed couplings 79 and 80, which permit rotation of the shafts 72 and 74. An extension joint 81 is provided in the pipe 76 between the shafts 72 and 74 to permit displacement of the shafts when the distance between the rollers is changed. The hollow shaft 73 and 75, on the other side of the machine, are connected to the inlet 82 of the generator 77 in a similar manner by means of sealed couplings 83 and 84 and extension joint 85.

On one side of the rollers, air nozzles 86 and 87 are disposed through the side of the machine so as to direct blasts of hot air across the upper and lower faces of the veneers as they emerge from the rollers. These nozzles are connected to the hot-air generator 71 by means of a pipe 88.

The following examples will further illustrate this invention and the manner in which it may be practiced:

*Example 1.*—Air-dry veneer or thin lumber containing any amount of moisture up to the fiber-saturation point (about 30 percent moisture content) is heated in a drier to a temperature of 200° F. to 300° F. under such conditions that no appreciable drying is effected. This generally requires circulation of air having a relative humidity of 75 percent or more. These veneers are then removed from the drier and directly fed into the apparatus, such as illustrated in Figures 1, 2, and 3, between the compression rollers thereof, with the clearance between the rollers set at about one-half the thickness of the veneer. As the veneers pass between the rollers, they are immersed in the treating bath, which may, by way of illustration, consist of a 50 percent aqueous solution of a phenol-formaldehyde resin-forming mix. After the veneer has been held submerged in the solution for about one minute, it recovers substantially completely from the compression and soaks in the solution. The veneer may then be removed from the treating bath.

*Example 2.*—Green, water-soaked veneer as it comes from the cutter knives or thin, green lumber prior to seasoning having a moisture content above the fiber-saturation point is first passed through a veneer drier, preferably a continuous drier to heat the veneer to about 200° F. without preventing any drying which may normally take place. The veneers are then fed directly from the drier to a device such as that illustrated in Figures 5 to 8, inclusive, in which the pressure rollers are set to compress the veneer to half its original thickness, the while permitting hot air to blow across the faces of the veneer through the nozzles 86 and 87 to remove any expressed water from the surface of the veneers. Promptly, upon removal from this operation, the veneers are fed to the apparatus, illustrated in Figures 1, 2, and 3, in a manner similar to that explained above in Example 1.

Instead of using phenol-formaldehyde resin-forming mix, other types of aqueous solutions may be used. Examples of other resin-forming mixes are urea-formaldehyde, melamine-formaldehyde, and phenol-furfural. Also, inorganic fire-retardant salts may be used, such as monoammonium acid phosphate, diammonium acid phosphate, and other phosphates, borates, and so forth. A number of toxic salts may also be used, such as zinc chloride, sodium fluoride, sodium arsenate, and other commercial mix salts and organic compounds. These examples may be used in any desired concentration.

A number of different types of preheating devices to plasticize the wood can be used. The heating can be done with steam, hot air, or with hot rollers or hot plates. When steam is used, it should be dry steam to avoid undue capillary condensation in the wood. Preheating above the boiling point of water is feasible only for veneer containing water below the fiber-saturation point. Preheating above 300° F. is not desirable because of the imbrittling effect upon the wood.

In the drying of green veneer, it may be advan-

tageous, if the moisture content is relatively high, to put the veneer through the drying rollers before heating so as to avoid the expense of heating a large excess of free water.

The extent to which the wood is compressed in either the drying or treating rollers may vary, depending upon the amount of solution which it is desired to take up, and is limited only by the extent of the void volume of the wood. The fraction of the original thickness to which dry veneer can be compressed can be calculated by dividing the oven-dry specific gravity of the wood by 1.46. The fraction of the original thickness to which veneer at the fiber-saturation point can be compressed can be calculated by dividing the green specific gravity by 1.12.

The length of time the compressed veneer should remain immersed in the solution after having been compressed will vary with the species and the amount of solution that it is desired to take up. Spruce and cottonwood take up an adequate amount of solution for most purposes in about 10 seconds. Birch may require immersion for as long as 10 minutes.

Having thus described my invention, I claim:

1. The process comprising plasticizing with heat a water-soaked wood veneer, expressing and removing free water from the coarse capillary structure of the veneer to establish a void volume, thence simultaneously submerging the plasticized, dewatered veneer in an aqueous solution and passing it between compression rollers, thence holding the veneer in the solution to permit it to take up the solution as it recovers from the compression.

2. The process comprising plasticizing with heat at a temperature of 200° F. a water-soaked wood veneer, expressing and removing free water from the coarse capillary structure of the veneer to establish a void volume, thence simultaneously submerging the plasticized, dewatered veneer in an aqueous solution and passing it between compression rollers, thence holding the veneer in the solution to permit it to take up the solution as it recovers from the compression.

3. The process for impregnating water-soaked wood veneer with an aqueous solution comprising plasticizing it with heat, expressing and removing free water from the coarse capillary structure in an amount substantially comparable to the quantity of the solution with which it is desired to impregnate the veneer, thence simultaneously submerging the plasticized, dewatered veneer in an aqueous solution and passing it between compression rollers, thence holding the veneer in the solution to permit it to take up the solution as it recovers from the compression.

4. Apparatus comprising a tank, co-acting compression rollers mounted on the tank, means for adjusting the clearance between said rollers, means for rotatably driving said rollers, the clearance between said rollers being disposed below the maximum liquid level of the tank, and means for cooling the liquid in the tank, said cooling means being disposed adjacent the rollers.

5. The process comprising plasticizing with heat a wood veneer having a void volume, thence simultaneously submerging the plasticized veneer in an aqueous solution cooler than the veneer and passing it between compression rollers, thence holding the veneer in the solution to permit it to take up the solution as it recovers from the compression.

ALFRED J. STAMM.